

Oct. 19, 1926.

R. G. COATES

1,603,662

INGOT

Original Filed August 17, 1923



*Fig. 1.*



*Fig. 2.*

INVENTOR

Ray G. Coates  
BY  
George Ramsey  
his ATTORNEY

## UNITED STATES PATENT OFFICE.

RAY G. COATES, OF PASADENA, CALIFORNIA, ASSIGNOR, BY MESNE ASSIGNMENTS, OF ONE-HALF TO ESTATE OF H. G. HAMILTON, DECEASED, LATE OF YOUNGSTOWN, OHIO.

## INGOT.

Original application filed August 17, 1923, Serial No. 657,855. Divided and this application filed October 4, 1924. Serial No. 741,527.

This invention relates broadly to metallurgy and more especially to improvements in ingots.

The present application is a division of my prior application Serial Number 657,855 on "Method and apparatus for casting ingots" filed August 17, 1923, which application matured into Patent No. 1,553,849, September 15, 1925.

Heretofore, in the art, it has been customary to cast top poured ingots one at a time so that a number of ingots from a single ladle of molten metal are individually quickly cast by quickly filling the vertical chill moulds in series. The time of casting a number of ingots is measured by the interval between beginning of casting and when the casting is ended; and the time for filling each mould is therefore a unitary divisible part of this interval, which is equal to dividing the total interval of casting into a number of individual time periods equal in number to the number of ingots being cast.

In the molten production of steel, the charges are usually poured into ladles which will hold from fifty to one hundred tons of molten steel. The length of time of pouring from the ladle is controlled by the period that the steel in the ladle will remain molten, since it must in any case be discharged before it freezes in the ladle. Where a number of ingot moulds are set up for casting, as is common in the art, it is necessary to move the ladle from one mould to another or to move the moulds past the pouring station by means of a train of cars on which the moulds are carried. Since the time for discharging the ladle is fixed and since the moulds must be filled either individually or in small groups, the ingots last cast will be cast from colder metal than those first cast, and the time of casting per individual ingot is very short as compared to the total time of ladle discharge; that is, when the first mould is filled, the filling operation as to that mould is completed, and the first mould has commenced to solid-

ify before the last ingot cast from the charge has been poured.

This rapid pouring necessarily fills the mould long before the mass of metal in the mould substantially freezes and the freezing will be largely from the sides toward the center with a relatively large pool of molten metal in the center of the mould. This pool, which is substantially the entire, very gradually freezes from the sides inward and from the bottom up. During this operation, gases which are forced from the freezing steel into the molten pool must rise through the molten metal which is slowly congealing and these gases produce cavities, pipes, etc. The metalloids of this large freezing pool are being left in the solution of the molten mass to continually enrich the last metal to freeze, so that it contains a much larger content of metalloids than the first metal to freeze at the sides, and bottom of the ingot. Furthermore, since the freezing is from the side walls inwardly, contractional cavities and pipes also occur in these quickly poured masses when they freeze.

The present invention comprises an ingot which is produced by very slowly poured metal so that the freezing occurs from the bottom upward and a shallow pool of molten material only is maintained in the mould as the ingot is being formed. This permits the gases to escape readily through the shallow pool and allows the shallow pool of metal to fill in any contractional cavities that tend to form so that the resultant ingot is substantially sound throughout its length. It is in effect formed by maintaining a relatively small amount of molten steel on the upper end of a constantly freezing upwardly growing column of solid metal.

Since there is only a shallow pool of metal being frozen and since the freezing progresses rapidly relatively to the pouring the metalloids are frozen in throughout the length of the ingot and are not thrown out in freezing as where a very large mass

of hot metal is cooled as in the prior art.

My prior Patent No. 1,553,849 above referred to discloses and claims one form of apparatus and method for producing the present ingot and for the purposes of explanation here, it may be stated that the ingot is manufactured by slowly feeding metal in a plurality of moulds during the entire discharge of the metal from the ladle so that a series of moulds are simultaneously being filled from the ladle in such manner that a relatively long period of time occurs between the beginning of casting and the end of casting, which period of time is substantially equal for all of the moulds in the series. This time may equal the complete time necessary to discharge the entire ladle, where a group of moulds having a group capacity equal to the ladle are being utilized.

The ingot comprising this invention is one in which the iso-crystallization zones are a plurality of cupped-shaped zones superimposed one upon the other throughout the vertical length of the ingot. Where a series of ingots are formed at one time, each of the series will have substantially the same corresponding iso-crystallization cupped zones, and have substantially the same chemical and physical characteristics.

In view of the foregoing, it may be stated that the principal object of the present invention is an ingot having a plurality of shallow iso-crystallization zones superimposed one upon the other throughout the vertical length of the ingot.

Another object of the present invention is an ingot of steel and the like comprising a substantially solid mass of metal having shallow iso-crystallization zones throughout the length thereof.

A further object of the present invention is an ingot of steel and the like in which the metal at the base of the ingot is of the character of the metal first poured from the ladle and the metal at the top of the ingot is of the character of the metal last poured from the ladle.

A still further object of the present invention is a series of ingots comprising articles of manufacture with each of the series comprising a portion of a large mass of metal poured from a common ladle and in which the bases of said ingots comprise metal first poured from the ladle and the tops of the ingots comprise metal last poured from the ladle.

Figure 1 of the drawing illustrates a longitudinal section through an ingot in accordance with the present invention in which the theoretical zones of iso-crystallization are represented by curved lines showing the form of the cupped-zones through substantially the center of the ingot.

Figure 2 is a sectional view through a

plurality of vertical ingot moulds illustrating the formation of ingots comprising the present invention.

Referring now to the drawings, and more especially to Figure 2, which illustrates the formation of ingots comprising the present invention. Vertical ingot moulds 1 are set on a casting stool 2 and the molten metal, for example molten steel, is run into the moulds in small streams 4 in any suitable way. These small streams are parts of a charge in a ladle, which charge is so subdivided that the streams 4 may continue throughout substantially the complete ladle full of molten metal. These streams are of such size as to slowly fill the matrix portion 5 of the moulds and permit solidification of the ingots to substantially follow up the filling of the mould so that the metal in the matrix of the moulds will comprise substantially solidified portions 6 and shallow pools 7. The rate of the flow of the streams 4 is maintained in such manner that the solidification follows up the filling of the mold.

Figure 1 illustrates a cross-section through an ingot 8 formed in accordance with the present invention and in which substantially parallel cupped iso-crystallization zones are illustrated by lines 9. These zones of course blend one into the other without definite demarkation, but are illustrated by definite lines as a matter of convenience. Preferably, ingots are cast simultaneously in groups and in such manner that each ingot is poured in substantially the same period of time from substantially the same quality of steel or metal so that each ingot in the series or group will have substantially the same characteristics.

The method and apparatus for producing the ingot is disclosed and claimed in my original application, filed August 17, 1923 and the present application therefore is limited to the ingot itself.

Having thus described my invention, what I claim is:

1. An article of manufacture comprising an ingot of steel having iso-crystallization zones comprising shallow cupped zones, with the concave portion of the cup being toward one end of the ingot, and having the metalloid content distributed substantially equally throughout the ingot.

2. An article of manufacture comprising an ingot of ferrous metal having the characteristic of a plurality of cupped zones of iso-crystallization with the zones substantially parallel and with the said zones extending transversely of the longitudinal axis of the ingot, and with the metalloids distributed substantially equally throughout the ingot.

3. An ingot of ferrous metal comprising an elongated mass having substantially sim-

ilar cupped zones of iso-crystallization superimposed one upon the other from one end of the ingot to the other, and with the ingot comprising a solid mass of steel having substantially uniform physical and chemical characteristics throughout.

4. An article of manufacture comprising an ingot of ferrous metal having a substan-

tially solid interior with a plurality of cupped zones of iso-crystallization and the deepest portion of said cups being substantially on the vertical axis of said ingot and with the metalloid content of the ingot being substantially uniform in a transverse section of the ingot.

RAY G. COATES.